

March 29, 1966

W. L. JACKSON

3,243,338

FLEXIBLE ELASTOMERIC ARTICLES AND REINFORCEMENT THEREFOR

Filed Aug. 7, 1961



Fig. 1



Fig. 2



Fig. 3

INVENTOR

William Lewis Jackson

By Stevens Davis Miller & Mosher  
Attorneys

## 1

3,243,338

**FLEXIBLE ELASTOMERIC ARTICLES AND  
REINFORCEMENT THEREFOR**

William Lewis Jackson, Whitworth, near Rochdale, England, assignor to Dunlop Tire and Rubber Corporation, Buffalo, N.Y., a corporation of New York

Filed Aug. 7, 1961, Ser. No. 129,903

7 Claims. (Cl. 161—58)

This invention relates to flexible elastomeric articles having improved reinforcement and to a pneumatic tire having an improved breaker strip.

According to the invention flexible elastomeric articles have embedded therein textile cords which comprise cords of filaments helically wrapped with yarn.

The invention also includes a textile reinforcement having a sheet of parallel cords which comprise filaments helically wrapped with yarn.

The yarn wrapping of the cords which surrounds the inner filaments, also referred to herein as the core of the cord, confers fatigue resistant properties on the cord and on the flexible elastomeric articles wherein the cord is embedded, and increases the stiffness conferred by the filaments.

In applications where stiffness is required in the reinforcement, as in the breaker strips of pneumatic tires for motor road vehicles, this is enhanced by increasing the size of the core and of the filaments which make up the cord, by arranging the filaments so that the cord is substantially circular in cross-section, by minimizing the twist of the filaments and increasing the binding effect of the wrapping, for instance by increasing the tension in the wrapping yarn and by increasing the number of the wrapping yarns, preferably by providing two superposed layers of wrapping yarns which are symmetrically disposed and arranged along the core. The filaments used in the core may be bonded together by an adhesive.

For use as a breaker strip the stiffness conferred by using cords as described is sufficient to resist lateral distortion of the tread.

Lateral distortion occurs at the region of contact between the road and the tire when the vehicle to which the tire is fitted is cornering. This distortion causes an extension at one side of the tread and a corresponding compression at the other side. It has been confirmed by experiment that for maximum stiffness and stability the resistance to compression should be substantially equated with the resistance to extension and while steel cords possess these characteristics they are not inherent in textile materials.

The resistance of filaments to compression and consequent buckling increases as the fourth power of the filament thickness, other things being equal, and the resistance to compression is closely allied to the increase in stiffness in the reinforcement according to the invention.

A breaker strip may be constructed from a sheet of parallel cords of above about 3,500 denier comprising a core having as low a twist as is consistent with satisfactory processing, for instance 1 to 3 turns per inch, formed of filaments having a weight per unit length greater than about 6 denier per filament, each cord having a breaking strength of more than about 30 pounds, i.e., a tenacity of more than about 3 grams per denier. The filaments may conveniently be employed in three core

## 2

yarns of about 1,650 denier each; more core yarns may be employed if desired but two should preferably not be used since they give a flat cord with increased liability to buckling under compression.

The stiffer man made filaments, such as rayon having 20 denier filaments, are liable to breakage in use and synthetic filaments having greater resilience and less extensibility usually give increased fatigue resistance. Synthetic filaments for use in a breaker strip having two sheets of cords preferably have an extensibility of not greater than 1 percent under a load of 10 lbs. Reduction of stiffness in use is caused at least in part by the cords being forced into an undulating configuration when the breaker strip is deflected with stretching and breakage of the filaments at the turning points of the undulations. Increasing the diameter of the cords usually increases the fatigue resistance since the wave length of the undulations is increased with a consequent reduction in the points at which the filaments are weakened.

Preferably, the core is wrapped with two layers of wrapper yarns, one wrapped in S direction and the other in Z direction, both having a twist greater than 12 turns per inch and a suitable weight being 840 denier.

In general the degree of twist of the wrapper yarns about the core should be sufficient to ensure that the angle between the wrapper yarns and the longitudinal axis of the cord is greater than 40 degrees. A higher degree of wrapper twist is required for thin cords than for thicker cords.

The cord may be produced by passing the filaments of the core through a hollow spindle on which a package of wrapper yarn is mounted and wrapping the yarn from the revolving package by means of a ring and traveller as the core is progressed through the spindle. A twist in the core of 2 turns per inch was found sufficient to control the passage of the filaments through the spindle.

The cords may be embedded in the tire carcass or in a separate breaker strip preparatory to inclusion in a tire carcass during molding thereof. It is convenient to employ the cords in the form of a woven reinforcement sheet having a number of parallel cords which are held in the sheet by transverse binder threads. The sheet is preferably dipped in an adhesive bath, for instance latex, and dried before use and the filaments, or bundles of filaments may be similarly treated prior to wrapping.

The invention will be further described with reference to the accompanying drawings in which:

FIG. 1 shows a textile cord having filaments helically wrapped with yarn,

FIG. 2 shows a textile reinforcement having two sheets of parallel cords, shown separated for clarity and

FIG. 3 shows a pneumatic tire having a breaker strip comprising two sheets of parallel cords.

The textile cord 1 of FIG. 1 has a core of seven symmetrically bunched 840 denier nylon filaments 2. The filaments have a twist of 2 turns per inch and the core a twist of 0.5 turn per inch. The core was wrapped with two wrapper yarns 3, 4 of mixed 300 denier rayon and 210 denier nylon at an angle of 75 degrees with respect to the longitudinal axis of the cord.

The textile cords 1 were assembled in side by side relationship in sheets and dipped in latex. Strips of sheet 5, 6 shown in FIG. 2 were cut and the strips 5 and 6 were adhered together so as to form a breaker strip with the cords 1 of the respective strips of sheet inclined in

opposed directions symmetrically with respect to the longitudinal axis of the strips.

The breaker strip was incorporated in a pneumatic tire 7 as shown in FIG. 3.

Cords having the following construction were prepared from filaments having the ply/denier values noted and the physical properties of the cords were evaluated. The following results were obtained.

Breaker strips having sheets with 16 cords per inch were incorporated in tires and the cornering force at 4 degrees slip was obtained before and after running the tires for 500 miles. The extensibility of the cord is given in the following table by the elongation under a 10 lb. load, and figures are given showing the load-extension ratios of the breaker strips.

Table 1

| Cord | Core                                                  | Core twist, t.p.i. | Wrapper                       | Strength in tension (lb.) | Diameter (in.) | Denier |
|------|-------------------------------------------------------|--------------------|-------------------------------|---------------------------|----------------|--------|
| 1    | Steel*                                                | 1.0                |                               | 155                       | 0.038          | 24,000 |
| 2    | 3/1650 rayon having 2.3 denier filaments <sup>a</sup> | 9S/9Z              |                               | 35                        | 0.034          | 5,600  |
| 3    | 3/1650 rayon having 20 denier filaments               | 1.5Z               | 2/840 nylon                   | 30                        | 0.044          | 11,000 |
| 4    | do                                                    | 1.5Z               | 4/840                         | 30                        | 0.065          | 19,900 |
| 5    | 7/1650 rayon having 20 denier filaments               | 1.5Z               | 2/840                         | 70                        | 0.065          | 23,000 |
| 6    | 1/3,200 terylene                                      | 1.0Z               | 4/1100 rayon                  | 44                        | 0.053          | 14,500 |
| 7    | 3/3,200 terylene                                      | 1.0Z               | 2/840 nylon                   | 120                       |                |        |
| 8    | 1/3,200 terylene                                      | 1.0Z               | 2/600 rayon                   | 44                        | 0.0386         | 7,160  |
| 9    | do                                                    | 1.0Z               | 4/600 rayon                   | 44                        | 0.0480         | 11,990 |
| 10   | 7/840 nylon                                           | 0.5Z               | 2/mixed: 300 rayon, 210 nylon | 105                       | 0.0496         | 10,330 |
| 11   | do                                                    | 0.5Z               | 4/mixed: 300 rayon, 210 nylon | 105                       | 0.0592         | 15,550 |
| 12   | 3/1650 having 2.3 denier filaments                    | 9S/9Z              | 2/840 nylon                   | 35                        | 0.0510         | 12,380 |

\*Included for purposes of comparison.

Sheets of parallel cords of the respective constructions noted in Table I were embedded in rubber breaker strips, a pair of sheets being provided in each face of the strips which were half an inch thick. The cords of the pairs of sheets were inclined at +20° and -20° respectively to the length of the strip and the cord density in the sheets was 80 percent of the number of cords which could be included. The stiffness of the breaker strip was determined by measuring the deflection of a three inch wide section of the strip under a load of 150 lb. The following results were noted:

Table 2

| Cord | Stiffness of strip | Properties of sheets of cord in sample face |                             |
|------|--------------------|---------------------------------------------|-----------------------------|
|      |                    | Strength per inch width (lb.) in tension    | Cord density (ends per in.) |
| 1    | 16                 | 3,200                                       | 21                          |
| 2    | 4                  | 800                                         | 23                          |
| 3*   | 6                  | 1,600                                       | 2 x 23 50                   |
| 3    | 10                 | 540                                         | 18                          |
| 4    | 16                 | 360                                         | 12                          |
| 5    | 40                 | 840                                         | 12                          |
| 6    | 12                 | 660                                         | 15                          |
| 7    | 10                 |                                             |                             |
| 8    | 12.9               | 925                                         | 21                          |
| 9    | 11.1               | 705                                         | 16                          |
| 10   | 21.7               | 1,680                                       | 16                          |
| 11   | 18.2               | 1,470                                       | 14                          |
| 12   | 8.8                | 560                                         | 16                          |

\*Two pairs of sheets were included in each face of the strip.

Breaker strips having sheets of steel cord 1 and wrapped textile cords 3 of Tables 1 and 2 and conventional breaker strips having a stiffness of 3 containing a standard tire cord were incorporated in tires and cornering force-slip angle curves obtained. The curves for the respective tires showed maximum difference at a slip angle of 2 degrees, the corresponding cornering forces being 235 lbs., 200 lbs. and 140 lbs., respectively. The ratio of the stiffnesses of the breaker strips containing steel and wrapped textile cords respectively with respect to that of the conventional breaker strip gives a substantially accurate forecast of the initial stiffness conferred upon tires incorporating the breaker strips. At a slip angle of 2 degrees the cornering force ratios :235/140=1.68 and 200/140=1.43 are in substantial agreement with the cube root of the stiffness ratio.

Table 3

| Cord of Table 1 | Cord extensibility, percent | No. of sheets in breaker strip | Tire size | Load extension ratio of breaker strip | Cornering force, lbs. |                  |
|-----------------|-----------------------------|--------------------------------|-----------|---------------------------------------|-----------------------|------------------|
|                 |                             |                                |           |                                       | As new                | 500 miles        |
| 1*              | 0.40                        | 2                              | 6.5-15    | 0.40                                  | 465                   | 440              |
| 10*             | 0.50                        | 2                              |           | 0.50                                  |                       |                  |
| 10              | 0.75                        | 2                              | 6.5-15    | 0.75                                  | <sup>b</sup> 370      | <sup>b</sup> 370 |
| 2               | 2.2                         | 6                              | 165-38    | 0.73                                  | <sup>c</sup> 294      | <sup>c</sup> 294 |
| 2               | 2.2                         | 4                              | 165-15    | 1.1                                   | <sup>c</sup> 260      | <sup>c</sup> 260 |
| Nil*            | 7.5                         | <sup>d</sup> Nil               | 5.90-15   | 7.5                                   | <sup>e</sup> 220      |                  |

\*Included for purposes of comparison.

<sup>a</sup> This cord was made up as cord 10, the nylon of the core being subjected to no stretching.

<sup>b</sup> Proportional cornering force estimated from sheets having 13 cords per inch.

<sup>c</sup> Proportional cornering force estimated from tire treads and breaker strips which were 50 percent wider than those of the other tires.

<sup>d</sup> This tire had four casing plies having cords biased at some 36°, the other tires having two ply casings of heavier cords disposed at 90°.

Having now described my invention, what I claim is:

1. In a flexible elastomeric article, a reinforcement comprising a sheet of parallel cords, each of said cords comprising a plurality of rigid filaments forming a core and having a twist of less than 3 turns per inch and a denier greater than 6, and at least two layers of yarns tightly wound over said filaments and extending at an acute angle with respect to the transverse axis of said cord.

2. The article of claim 1 wherein said cords each have a denier greater than 3500 and a breaking strength of at least 30 pounds.

3. The article of claim 1 wherein adjacent layers of 65 yarns are wrapped in S direction and Z direction respectively.

4. The article of claim 1 wherein the filaments are of nylon and the yarns are of a mixture of nylon and rayon.

5. The article of claim 1 wherein the filaments are of synthetic material and have an extensibility of not greater than 1 percent under a load of 10 pounds.

6. The article of claim 1 wherein there are at least two sheets of parallel cords.

7. The article of claim 6 wherein adjacent sheets of 75 said cords are adhered together with their cords being

inclined in opposed directions symmetrically with respect to the longitudinal axis of the reinforcement.

**References Cited by the Examiner**

UNITED STATES PATENTS

|           |        |              |         |
|-----------|--------|--------------|---------|
| 271,548   | 1/1893 | Trott et al. | 174—122 |
| 1,462,453 | 7/1923 | Lerch        | 152—361 |
| 2,087,303 | 7/1937 | Rosch et al. | 174—122 |
| 2,468,304 | 4/1949 | Musselman    | 161—176 |
| 2,498,859 | 2/1950 | Lessig       | 152—355 |
| 2,598,033 | 5/1952 | Bourdon      | 57—144  |

5

|           |        |              |         |
|-----------|--------|--------------|---------|
| 2,755,214 | 7/1956 | Lyons et al. | 154—52  |
| 2,782,830 | 2/1957 | Wallace      | 153—355 |
| 2,786,507 | 3/1957 | Howe et al.  | 152—355 |
| 2,974,559 | 3/1961 | Coggi        | 161—176 |

FOREIGN PATENTS

|                                                  |         |         |
|--------------------------------------------------|---------|---------|
| 1,218,661                                        | 12/1959 | France. |
| ALEXANDER WYMAN, Primary Examiner.               |         |         |
| EARL M. BERGERT, Examiner.                       |         |         |
| L. T. PIRKEY, G. D. MORRIS, Assistant Examiners. |         |         |